

# United States Patent

[11] 3,601,645

|      |           |                                             |           |         |                    |           |
|------|-----------|---------------------------------------------|-----------|---------|--------------------|-----------|
| [72] | Inventor  | Colin Whiteheart<br>Morden, England         | 2,353,047 | 7/1944  | Lannert.....       | 310/251   |
| [21] | Appl. No. | 825,305                                     | 1,067,003 | 7/1913  | Deats et al. ....  | 310/253   |
| [22] | Filed     | May 16, 1969                                | 2,989,490 | 6/1961  | Ramadanoff .....   | 310/253 X |
| [45] | Patented  | Aug. 24, 1971                               | 1,633,815 | 6/1927  | Kelley .....       | 310/249   |
| [73] | Assignee  | Marganite Carbon Limited<br>London, England | 2,319,240 | 5/1943  | Larsen et al. .... | 310/252 X |
| [32] | Priority  | May 23, 1968                                | 1,708,192 | 4/1929  | Sherwood.....      | 310/249   |
| [33] |           | Great Britain                               | 661,669   | 11/1900 | Rohrer .....       | 310/249   |
| [31] |           | 24,637/68                                   | 764,391   | 7/1904  | Street.....        | 310/249   |
|      |           |                                             | 1,712,477 | 5/1929  | Hediger.....       | 310/249   |
|      |           |                                             | 2,092,627 | 9/1937  | Adams .....        | 310/249   |
|      |           |                                             | 2,098,062 | 11/1937 | Palmer .....       | 310/249   |

[54] **ELECTRICAL CONTACT BRUSHES**  
10 Claims, 7 Drawing Figs.

[52] U.S. Cl. .... 310/249,  
29/630 E, 310/251, 310/252  
[51] Int. Cl. .... H01r 39/36  
[50] Field of Search. .... 219/226;  
245/247; 310/249, 251, 252, 253

[56] **References Cited**  
UNITED STATES PATENTS  
1,053,881 2/1913 Scott et al. .... 310/251

Primary Examiner—D. F. Duggan  
Assistant Examiner—B. A. Reynolds  
Attorney—Baldwin, Wight & Brown

**ABSTRACT:** An electrical brush comprises a metal-and-carbon containing body and a metallic layer to which an electrical conductor is or may be secured and electrically connected. The metal-and-carbon containing body is sintered with the metallic layer in an area which is greater than the area at the connection of the electrical conductor to the layer.



PATENTED AUG 24 1971

3,601,645



Fig.1.

Fig.2.



Fig.3.

Fig.4.

Fig.5.



Fig.6.

Fig.7

Inventor:

Colin Whiteheart

By Baldwin Wright Miller & Brown  
Attorneys

**ELECTRICAL CONTACT BRUSHES**

This invention relates to electrical contact brushes and to the manner in which a flexible electrical conductor is attached to the body of the brush.

It is known to attach a flexible conductor to a brush by inserting the conductor in a hole formed in the body of the brush and thereafter securing the conductor within the hole by means of, for example, solder or compressed metal, or a rivet, or by swaging the brush around the conductor. These methods are well established but they are not all universally applicable; consequently a particular method of attachment must be selected for a particular brush design or construction. For example, it is very difficult to drill a suitable hole if the brush is very small. Also the various methods have their own particular disadvantages. The use of compressed powders in a hole may not provide adequate securing strength when the conductor is subjected to intermittent vibration and shock. Soldering presents problem due to the shrinkage of the material when the solder cools. Swaging raises the brush material density in the area at which the swaging takes place, and this represents a waste of expensive copper, for example, and it can also lead to disintegration of the brush material at the swaging area.

The present invention seeks to overcome these disadvantages.

According to the present invention an electrical contact brush comprises a metal-and-carbon containing body, a metallic layer sintered with said body, and electrical conductor means secured to said metallic layer and electrically connected therewith, said metallic layer having a greater tensile strength than that of said body.

The brush body may be made of a number of materials known in the art of electrical brush manufacture. Thus it may be selected from a wide range of materials going from a mixture of carbon with various metals or alloys (for example copper or copper with one or more additives such as lead, tin, manganese or silver), carbon/metal mixtures containing small quantities of other additives such as nonconducting abrasives and lubricants including molybdenum disulfide and P.T.F.E., i.e. polytetrafluoroethylene, through to metals containing only small amounts of carbon and/or other additives.

The main purpose of this invention is to overcome the problems encountered with brush designs wherein there is a weakness in the area of the junction between the body and the flexible conductor and particularly in the body portion immediately surrounding the junction. Therefore, whilst the invention might be applicable to almost all brushes, it is particularly concerned with brushes whose body construction is such that problems have been encountered in usage due to fracture near the junction of the body with the flexible conductor.

Thus the metallic material of the layer sintered onto the body is chosen to have a greater tensile strength than the material of the body (which itself may contain a large proportion of metal), and the area of contact between the metallic layer and the body should be larger than the area of contact between the flexible conductor and the metallic layer, thereby effectively spreading the load over a relatively large area of the body if any jerks are applied to the flexible conductor.

In one preferred embodiment of the invention the metallic layer effectively covers the face of the body of the brush opposite to the working (electrical contact) face.

Examples of the present invention will now be described with reference to the accompanying drawing in which:

FIG. 1 is a side view of one embodiment of an electrical contact brush,

FIG. 2 is a view, in cross section, of another embodiment of an electrical contact brush, and

FIGS. 3-7 illustrates various steps in the manufacture of an electrical contact brush.

In the figures an electrical contact brush comprises a body 1 having attached thereto a metallic layer 2 to which is secured a flexible electrical conductor 3. The brush body 1 is com-

posed primarily of a metal and graphite and the metal can be, for example, copper together with alloy constituents known in the art. The metallic layer 2 can be composed of, for example, copper or iron, or a mixture thereof but the invention is not limited to the use of such metals. The flexible conductor 3 may be formed from thin electrically conductive metal strands of, for example, copper. The strands can, of course, be formed from any other suitable metal.

In the example illustrated in FIG. 1 the flexible electrical conductor 3 is attached to a surface of the metal layer 2 by welding. The welded joint is indicated at 4. It is preferred that the welded joint is made by using a pressure-resistance welding technique.

In FIG. 2 the flexible conductor 3 is secured to the metal layer 2 by forming a bore in the layer 2 and thereafter securing one end of the flexible conductor within the bore by tamping with, for example, copper particles 6.

Although not illustrated the flexible conductor 3 can, if desired, be placed in the bore and thereafter soldered to the metallic layer 2.

The brush body 1 is composed primarily of a metal and a graphite, and the metal may be copper with alloy constituents known in the art. Copper, or any other suitable metal can be present up to 95 percent of the total brush composition. A wide variety of materials may be used for the brush body, for example, compositions of metal and graphite in the range of from 25 percent copper, 75 percent graphite to 95 percent copper, 5 percent graphite, and the compositions may include lead, tin, zinc or a combination of these up to about 15 percent of the total composition so that, at the extreme, the brush composition may consist of 95 percent metal or alloy and 5 percent graphite. It will thus be realized that the actual brush materials themselves are not of prime importance but the present invention is particularly useful when it is necessary to attach a flexible copper conductor to a brush containing a major proportion of metal.

It is arranged that the surface area of contact between the metallic layer 2 and the brush body 1 is larger than that between the flexible conductor 3 and the metal layer 2. With this arrangement should the flexible conductor 3 be subjected to any form of tensile loading, the load per unit area on the body is comparatively reduced and certainly less than what it would be if the conductor were attached directly to the body.

It is preferred that the metallic layer 2 is formed and attached to the brush body 1 by cocompacting and cosintering the layer material together with the brush body material.

The compacting and sintering processes are illustrated schematically in FIGS. 3-7. FIG. 3 represents a compaction press which includes a die 7 having a pair of reciprocal plungers 8 and 9. Metallic powders to form the brush body 1 are placed in the die as shown in FIG. 4. The bottom plunger 8 is then lowered by a specified amount. Powders which constitute the metallic layer 2 are then put in the die 7 on top of the constituent powders of the brush body 1. This is shown in FIG. 6. The top plunger 9 is then brought down to compress and so compact the powders together and the compacted constituents are then sintered at a suitable temperature for a suitable period of time.

In one particular example of the present invention the following metallic powders were blended together with a small amount of die lubricant, stearic acid (zinc stearate was also suitable as the die lubricant):

78 parts by weight of 100 mesh copper powder,  
10 parts by weight of 200 mesh lead powder,  
six parts by weight of 100 mesh manganese powder, and  
six parts by weight of 200 mesh natural graphite.

The mixture of powders was put into the die of a compaction press and on to the top of this powder was placed a measured quantity of 100 mesh reduced sponge iron powder to form a layer of 5 mm. depth. The powders were then cocompacted together at 10 tons per square inch pressure and were cosintered at 840° for 1 hour in a suitable protected atmosphere.

It should be noted that the powders forming the brush body 1 can be compressed before the powders constituting the metallic layer 2 are placed thereon. However, subsequent compaction does not provide a bond between the body and the layer as good as that of the first mentioned process. Accordingly, the first process is preferred.

The cocompacting and cosintering processes provide an excellent physical and electrical bond between the brush body and the metal layer. The joint between the flexible electrical conductor and the metallic layer, whether it be made by welding, tamping or soldering, is physically strong since the attachment is made between two metals. And since the surface area at the interface between the metallic layer and the brush body is larger than that between the flexible conductor and the layer any tensile loading applied to the flexible conductor will be distributed evenly over the rush at said interface.

What I claim is:

1. An electrical brush comprising a metal-and-carbon containing body, a metallic layer sintered with said body, said metallic layer comprising a metal other than any ingredient of said body, and electrical conductor means secured to said metallic layer and electrically connected therewith, said metallic layer having a greater tensile strength than that of said body.
2. An electrical brush according to claim 1 wherein the surface area of contact at the interface between said metallic layer and said body is greater than that between said metallic layer and said conductor means.

3. An electrical brush according to claim 1 wherein said conductor means comprises a flexible electrical conductor, said flexible conductor being secured integrally to said metallic layer.
4. An electrical brush according to claim 1 wherein said metallic layer consists essentially of a metal.
5. An electrical brush according to claim 4 wherein said metal is iron.
6. An electrical brush according to claim 1 wherein said metallic layer comprises copper.
7. An electrical brush according to claim 1 wherein said metallic layer consists essentially of a metal alloy.
8. An electrical brush according to claim 1 wherein said metallic layer consists essentially of a mixture of copper and iron.
9. An electrical brush according to claim 1 wherein said body is a composition essentially of copper and graphite in the range of from 25 percent copper, 75 percent graphite to 95 percent copper, 5 percent graphite.
10. An electrical brush comprising a body of sintered metal-and-carbon; a sintered metallic material layer, said metal-and-carbon of said body being cosintered with the metallic material of said layer, said metallic material layer comprising a metal other than any ingredient of said body; and electrical conductor means secured to said layer and electrically connected therewith, said layer having a greater tensile strength than said body.

30

35

40

45

50

55

60

65

70

75